

[54] **PROCESS FOR DRESSING AND PROVIDING  
LEATHER WITH AN ANTIMICROBIAL  
FINISH**

[75] Inventors: **Rosemarie Töpfl**, Dornach; **Max Schwank**, Basel; **Gerhard Hool**, Lupsingen, all of Switzerland

[73] Assignee: **Ciba-Geigy Corporation**, Ardsley, N.Y.

[22] Filed: **Dec. 5, 1974**

[21] Appl. No.: **529,887**

[30] **Foreign Application Priority Data**

Dec. 12, 1973 Switzerland..... 17402/73  
Dec. 12, 1973 Switzerland..... 17404/73

[52] U.S. Cl..... **427/386**; 427/389;  
427/390 R

[51] Int. Cl.<sup>2</sup> ..... **B05D 3/02**  
[58] Field of Search ..... 427/390, 391, 386, 389

[56] **References Cited**

UNITED STATES PATENTS

3,769,365 10/1973 Toepfl et al. ..... 260/834

Primary Examiner—Michael R. Lusignan  
Attorney, Agent, or Firm—Joseph G. Kolodny; Edward  
McC. Roberts; Prabodh I. Almaula

[57]

**ABSTRACT**

A process for dressing and providing leather with an antimicrobial finish is provided, which comprises treating the leather with aqueous preparations of (1) reaction products of (a) an epoxide that contains at least two epoxide groups in each molecule, (b) a fatty amine with 12 to 24 carbon atoms, (c) a dicarboxylic acid of the formula



wherein y is an integer from 1 to 13, optionally (d) an anhydride of an aromatic dicarboxylic acid with at least 8 carbon atoms, of an aliphatic monocarboxylic acid with at least 2 carbon atoms, or of an aliphatic dicarboxylic acid with at least 4 carbon atoms, (e) an aliphatic diol with 2 to 21 carbon atoms and/or (f) a difunctional compound which differs from components (a), (c), (d) and (e), which reaction products have been reacted or mixed or reacted and mixed with (2) aminoplast precondensates which contain alkyl ether groups, and subsequently drying the treated leather at elevated temperature.

The finished leather has good fastness properties, e.g. fastness to light, wet treatments and dry rubbing and also to ironing and creasing.

**28 Claims, No Drawings**

PROCESS FOR DRESSING AND PROVIDING  
LEATHER WITH AN ANTIMICROBIAL FINISH

The present invention provides a process for dressing and providing leather with an antimicrobial finish, which comprises treating the leather with aqueous or organic preparations of

1. reaction products of

- an epoxide that contains at least two epoxide groups in each molecule,
- a fatty amine with 12 to 24 carbon atoms,
- a dicarboxylic acid of the formula



wherein  $y$  is an integer from 1 to 13, optionally

- d. an anhydride of an aromatic dicarboxylic acid with at least 8 carbon atoms, of an aliphatic monocarboxylic acid with at least 2 carbon atoms, or of an aliphatic dicarboxylic acid with at least 4 carbon atoms,
- e. an aliphatic diol with 2 to 21 carbon atoms and/or
- f. a difunctional compound which differs from components (a), (c), (d) and (e), which reaction products have been reacted or mixed or reacted and mixed with

2. aminoplast precondensates which contain alkylether groups, and subsequently drying the treated leather at elevated temperature.

The preparations used according to the invention can be preferably aqueous emulsions or dispersions and optionally also organic solutions.

The epoxides of the component (a) are derived preferably from polyhydric phenols or polyphenols, e.g. resorcinol, or phenol-formaldehyde condensation products of the type of the resols or novolaks. Bis-phenols, e.g. bis(4-hydroxyphenyl)-methane and, above all, 2,2-bis(4'-hydroxyphenyl)-propane, are especially preferred starting compounds for the manufacture of the epoxides.

Compounds to be mentioned particularly are epoxides of 2,2-bis(4'-hydroxyphenyl)-propane which have an epoxide content of 1 to 6, particularly of 1.8 to 5.8 epoxy group equivalents/kg, but preferably at least 5 epoxy group equivalent/kg, and which have the formula



wherein  $z$  represents a mean number from 0 to 6, preferably from 0 to 2.2, and optionally also from 0 to 0.65. Such epoxides are obtained by reaction of epichlorohydrin with 2,2-bis(4'-hydroxyphenyl)-propane.

Mono-fatty amines with 12 to 24 carbon atoms have proved principally to be very suitable components (b). Usually these are amines of the formula



(II)

wherein  $x$  represents an integer from 11 to 23, preferably from 17 to 21. The amines are therefore, for example, laurylamine, palmitylamine, stearylamine, arachidylamine or behenylamine. Mixtures of these amines, like those obtainable in the form of commercial products, can also be used.

Alkylenedicarboxylic acids with 2 to 14 carbon atoms have proved advantageous as component (c). These are normally dicarboxylic acids of the formula



wherein  $y$  is an integer from 1 to 13, especially 1 to 5 and preferably 6 to 13.

15 Examples of suitable dicarboxylic acids for component (c) are accordingly oxalic, malonic, succinic, glutaric, adipic, pimelic, suberic, azelaic or sebacic acid, nonanedicarboxylic acid, decanedicarboxylic acid, undecanedicarboxylic acid or dodecanedicarboxylic acid.

20 Component (c) can be used by itself or optionally together with component (d), both components complementing each other.

As component (d) there is used preferably an anhydride of a monocyclic or bicyclic aromatic dicarboxylic acid with 8 to 12 carbon atoms or of an aliphatic dicarboxylic acid with 4 to 10 carbon atoms or of a monocarboxylic acid with at least 2 to 10 carbon atoms. Anhydrides of a monocyclic aromatic dicarboxylic acid with 8 to 10 carbon atoms have proved particularly advantageous. Particular interest attaches to phthalic anhydride which is optionally substituted by methyl.

25 Examples of suitable anhydrides for component (d) are accordingly acetic anhydride, maleic anhydride or phthalic anhydride.

30 35 If component (e) is used concurrently for the manufacture of the reaction products, the diols in question are preferably aliphatic diols with 2 to 21, preferably 2 to 6, carbon atoms the carbon chains of which are optionally interrupted by oxygen atoms. Particular interest in this connection attaches to alkylene diols with 2 to 6 carbon atoms or diethylene or triethylene glycol or also polyethylene or polypropylene glycols. Examples of alkylene diols with 2 to 6 carbon atoms which are used with particular advantage are ethylene 40 glycol, butanediol-1,4, neopentyl glycol or, preferably hexanediol-1,6.

45 As functional groups or atoms, the difunctional component (f), which is also optional, preferably contains

halogen atoms which are bonded to an alkyl radical, vinyl groups or carboxy ester groups or at most one epoxide, carboxy or hydroxy group together with another functional group or with another atom of the indicated type. In particular, these compounds are difunctional organic compounds that contain, as functional groups or atoms, alkyl-bonded chlorine or bromine atoms, vinyl groups or carboxy ester groups or at most one epoxide or carboxy group together with another functional group or another atom of the indicated type.

Particularly suitable difunctional organic compounds are aliphatic. They are, for example, epihalohydrins, such as epibromohydrin or, preferably epichlorohydrin.

Other possible difunctional compounds are, for example, glycerol dichlorohydrin, acrylic acid, methylolacrylic amide, acrylonitrile.

The aminoplast precondensates used as component (2) are desirably completely or, in particular, partially etherified methylol compounds of nitrogen-containing aminoplast formers, such as urea, thiourea, urea derivatives, e.g. ethylene urea, propylene urea or glyoxalmonourein.

Preferably, however, etherified methylolaminotriazines are used, for example alkyl ethers of highly methylolated melamine the alkyl radicals of which contain from 1 to 4 carbon atoms. Possible alkyl radicals include methyl, ethyl, n-propyl isopropyl, n-butyl and n-hexyl radicals. In addition to such alkyl radicals, yet further radicals, for example polyglycol radicals, can also be present in the molecule. Furthermore, n-butyl ethers of a highly methylolated melamine containing 2 to 3 n-butyl groups in the molecule are preferred. By highly methylolated melamines are meant in this context those with an average of at least 5, desirably about 5,5, methylol groups.

Alkyl ethers of methylolated urea, of the cited methylolated urea derivatives or preferably of methylolated aminotriazines are particularly suitable.

The component (2) can also be present simultaneously as mixture component or exclusively as mixture component, e.g. the preparations used in the process according to the invention can contain reaction products of components (a) to (f) and (2) or mixtures of component (2) with the reaction products of components (a) to (f) and (2) or mixtures of component (2) with the reaction products of components (a) to (f).

The manufacture of the reaction products can be carried out by methods which are known per se, wherein the components are reacted with one another in varying sequence. Desirably, the components (a) and (b) or (a) and (c) are first reacted with one another. The reaction of the component (c) with the already reacted components (a) and (b) can also be effected simultaneously, if appropriate, with the components (d), (e) and (f) or with component (2).

On the one hand, it is therefore possible to react the components (a), (b) and (c) initially with one another simultaneously and subsequently, if appropriate, to react the product with the components (d), (e), (f) and (2). In this modification of the process, the components (a), (b) and (c) are reacted with one another desirably at temperatures of 80°C to 120°C, preferably at 100°C, the proportions being generally so chosen that for an epoxide group equivalent of 1 there are used 0.05 to 0.7 amino group equivalent of component (b), 0.2 to 2.0, preferably 0.4 to 2.0, acid equivalents of component (c) and (d), 0.1 to 0.8, hydroxy group equivalent of component (e), 0.1 to 0.7 mole of component (f) and 10 to 80, preferably 30 to 60, percent by weight of component (2), based on the total weight of the components (a) to (f) and (2). If component (2) is used as mixture component, it can also be used in amounts of about 10 to 80, preferably 30 to 60, percent by weight, based on the total weight of the mixture of (1) and (2). The use of component (2) as mixture component without its simultaneous use as reaction component or its exclusive use as reaction component

for the manufacture of the reaction products is preferred.

On the other hand, it is also possible to react initially the components (a) and (b) alone with each other and then with component (c) and optionally in a third or fourth step with component (d), (e), (f) or (2). The manufacture of the reaction products of (a) and (b) in this second modification is also desirably carried out at temperatures of 80°C to 120°C, preferably at about 100°C. The reaction in the second step with component (c) is carried out desirably at 80°C to 110°C, preferably at about 100°C.

The reaction with components (d), (e), (f) and (2) is carried out normally at a temperature of 60°C to 100°C, preferably at about 100°C.

The reaction products that are obtained without using component (2) as reaction component can have as a rule an acid number of 5 to 100, preferably 15 to 60.

Suitable organic solvents in the presence of which the reaction products are manufactured are primarily water soluble organic solvents and desirably those that are infinitely miscible with water. Dioxan, isopropanol, ethanol and methanol, ethylene glycol-n-butyl ether (=n-butyl glycol), diethylene glycol monobutyl ether, dimethyl formamide, may be cited as examples.

Moreover, it is also possible to carry out the reaction in the presence of water-insoluble solvents, e.g. in hydrocarbons like petrol, benzene, toluene, xylene; halogenated hydrocarbons, e.g. methylene bromide, carbon tetrachloride, ethylene chloride, ethylene bromide, s-tetrachloroethane and especially also trichloroethylene.

The preparations used according to the invention contain reaction products that are manufactured using component (2) or they contain the reaction products in admixture with component (2). At least one aminoplast precondensate should be used either as reaction component (s) for the manufacture of the reaction products or as mixture component.

The preparations can contain, for example, the following reaction products or mixtures: reaction products of (a), (b), (c), (d), (f) and (2); reaction products of (a), (d), (c), (e), (f) and (2); mixtures of reaction products of components

(a), (b), (c), (d), (e), (f) and component (2);

(a), (b), (c), (e) and component (2);

(a), (b), (c), (f) and component (2).

The solids content in the preparations can be about 30 to 70 percent by weight.

The preparations are normally applied from an aqueous medium which contains the reaction products in emulsified form. An application can also be effected from organic solutions. To this end, the preparations of the reaction products are mixed with water and optionally with wetting agents and dispersants. The resultant stable, aqueous emulsions can have a pH of about 4 to 8, preferably 4 to 6. The solids content can be about 10 to 40 percent by weight. Examples of suitable wetting agents and dispersants are adducts of an alkyleneoxide, preferably ethylene oxide, and aliphatic or cycloaliphatic amines and alcohols of higher molecular weight, or fatty acids or fatty amides which optionally may be esterified at the hydroxy groups with polybasic or organic acids or, if they are nitrogen compounds, can also be quaternised. In addition, these compounds can also be reacted with further compounds in order to obtain e.g. a cross-linking effect.

Besides the emulsified reaction products or mixtures of the reaction products and the aminoplast precondensates, the application liquors can contain still other additives, e.g. acids or salts or also other finishing or improving agents. Phosphoric, sulphuric and hydrochloric acid or also oxalic, formic and acetic acid may be cited as examples of acids.

The amount of reaction product or mixture of reaction product and aminoplast precondensate (exclusive of solvent and water), based on the substrate, is desirably 1 to 10 g/m<sup>2</sup> for dressing leather. The application is effected as a rule at 20° to 100° C, preferably at room temperature, and by known methods, for example by immersion, spraying, brushing, padding or impregnating.

The treated leather is then dried, e.g. at temperature of 40° C to 70° C, preferably at 50° C to 60° C. The drying process normally lasts for about 30 to 120 minutes.

The leather to be finished can be of any desired provenance, but preferably so-called grained leather is used, viz. leather that is to be dressed on the grain side. The leather finishing can be carried out in two steps by applying the preparations according to the invention e.g. together with a dye or pigment suitable for colouring leather, drying the treated leather and then applying a colourless preparation that is able to impart e.g. an additional sheen to the coloured layer. The leather finished with these dressing agents has very good general fastness properties, in particular very good fastness to light, wet treatments and dry rubbing; it is also fast to ironing and creasing. The handle is also markedly improved. The dressed leather can therefore be termed as "easy-care". In the light of all its fastness properties, it is superior to leather that is dressed with polyurethanes or polyacrylates. In addition to the described effects an antimicrobial finish is imparted to the leather.

The microbial effect is attained against representatives of the Gram-positive and Gram-negative bacteria, for example against *Staphylococcus aureus*, *Escherichia coli* and *Proteus vulgaris* or against fungi, for example *Trichophyton mentagrophytes*.

The following Examples illustrate the invention, the parts and percentages being by weight.

#### EXAMPLE 1

A mixture of 196 g of an epoxide formed from 2,2-bis-(4'-hydroxyphenyl)-propane and epichlorohydrin (1 epoxide equivalent), 108 g of stearylamine (0.4 amino group equivalent) and 100 g of butyl glycol is stirred for 15 minutes at 100° C internal temperature. Then 73 g of adipic acid (1 acid equivalent) are added thereto and stirring is continued for 3 hours at 100° C internal temperature. Upon addition of 27.8 g of epichlorohydrin (0.3 mole), stirring is continued for a further 3 hours at 100° C internal temperature. The reaction mixture is subsequently diluted with 304.8 g of perchloroethylene and a 50% resin solution is obtained. Viscosity: 7740 cP. The viscosities are measured in a "Rotavisko" viscosimeter at 20° C (measuring instrument: NV)

Acid number: 85.

360 g of the above product are mixed with 150 g of an 80% solution of hexamethylolmelamine dibutyl and tributyl ether in butanol, 72 g of a 50% aqueous solution of an adduct of hydroabietyl alcohol and 200 moles of ethylene oxide (cross-linked) with 1% hexamethylene-1,6-diisocyanate and 29 g of a 50% aque-

ous solution of hydroabiethylamine and 70 moles of ethylene oxide. A finely disperse emulsion is obtained after addition of 389 g of water by stirring.

Resin content: 30 %, pH = 4.1.

#### EXAMPLE 2

A mixture of 49 g of an epoxide according to Example 1 (0.25 epoxide equivalent), 27 g of stearylamine (0.1 amino group equivalent) and 10 g of butyl alcohol is stirred for 1 hour at 100° C internal temperature. To this mixture are then added 7.8 g of neopentyl glycol (0.15 hydroxy group equivalent) and 14.8 g of succinic acid (0.25 acid equivalent). Then 7 g (0.075 mole) of epichlorohydrin are added thereto and stirring is continued for 2 hours at 100° C internal temperature. Subsequently 178 g of an 80% solution of hexamethylolmelamine dibutyl and tributyl ether in butanol, which has been diluted previously with 40 g of butyl glycol, are added over the course of 30 minutes and the reaction mixture is stirred for 1 hour at 100° C internal temperature. Dilution with 162.4 g of perchloroethylene yields a clear, 50% resin solution.

Acid number: 22. Viscosity: 12580 cP.

400 g of the above resin solution are mixed with 48 g of a 50% aqueous solution of an adduct of hydroabiethyl alcohol and 200 moles of ethylene oxide (cross-linked with 1% hexamethylene-1,6-diisocyanate) and 19 g of a 50% aqueous solution of an adduct of hydroabiethylamine and 70 moles of ethylene oxide. A finely disperse emulsion is obtained after addition of 533 g of water by stirring.

Resin content: 20%, pH: 4.1.

#### EXAMPLE 3

35 A mixture of 49 g of an epoxide according to Example 1 (0.25 epoxide equivalent), 27 g of stearylamine (0.1 amino group equivalent) and 10 g of butyl glycol is stirred for 1 hour at 100° C internal temperature. To this mixture are then added 7.8 g of neopentyl glycol (0.15 hydroxy group equivalent) and 13 g of malonic acid (0.25 acid equivalent) and stirring is continued for 3 hours at 100° C internal temperature. Then 7 g of epichlorohydrin (0.075 mole) are added and stirring is again continued for 2 hours at 100° C. Subsequently 175 g of an 80% solution of hexamethylolmelamine dibutyl and tributyl ether in butanol, which has previously been diluted with 40 g of butyl glycol, are added over the course of 30 minutes and the mixture is stirred for 1 hour at 100° C internal temperature.

50 Dilution with 158.8 g of perchloroethylene yields clear, 50% resin solution.

Acid number: 5.5. Viscosity: 720 cP.

400 g of the above resin solution are mixed with 48 g of a 50% aqueous solution of an adduct of hydroabiethyl alcohol and 200 moles of ethylene oxide (cross-linked with 1% hexamethylene-1,6-diisocyanate) and 19 g of a 50% aqueous solution of an adduct of hydroabiethylamine and 70 moles of ethylene oxide. A finely disperse emulsion is obtained after addition of 533 g of water by stirring.

Resin content: 20%, pH: 4.6.

#### EXAMPLE 4

65 A mixture of 196 g of an epoxide according to Example 1 (1 epoxide equivalent), 15.5 g of a mixture of 1-aminoeicosane and 1-aminodocosane (0.05 amino group equivalent) and 100 g of butyl glycol is stirred for 3 hours at 100° C internal temperature. To this

mixture are then added 102 g of adipic acid (1.4 acid equivalents) and stirring is continued for 3 hours at 100° C internal temperature. After addition of 9.25 g (0.1 mole) of epichlorohydrin stirring is again continued for 3 hours at room temperature and the product is subsequently diluted with 222.75 g of perchloroethylene. A clear, 50% solution is obtained.

Acid number: 93.6. Viscosity: 1040 cP.

360 g of the above product are mixed with 150 g of an 80% solution of hexamethylolmelamine dibutyl and tributyl ether in butanol, 72 g of a 50% aqueous solution of an adduct of hydroabietyl alcohol and 200 moles of ethylene oxide (cross-linked with 1% hexamethylene-1,6-diisocyanate) and 29 g of a 50% aqueous solution of hydroabietylamine and 70 moles of ethylene oxide. A finely disperse emulsion is obtained after addition of 389 g of water by stirring. Resin content: 30%, pH: 4.1.

#### EXAMPLE 5

A mixture of 196 g of an epoxide according to Example 1 (1 epoxide equivalent), 62 g of a mixture of 1-aminoeicosane and 1-amino-docosane (0.2 amino group equivalent) and 100 g of dimethyl formamide is stirred for 15 minutes at 100° C internal temperature. To this mixture are then added 31.2 g of neopentyl glycol (0.6 hydroxy group equivalent) and 73 g of adipic acid (1 acid equivalent) and stirring is continued for 3 hours at 100° C internal temperature. Then 27.8 g (0.3 mole) of epichlorohydrin are added and stirring is again continued for 3 hours at 100° C internal temperature. Dilution with 290 g of perchloroethylene yields a clear, 50% solution.

Acid number: 32. Viscosity: 1090 cP.

360 g of the above product are mixed with 150 g of an 80% solution of hexamethylolmelamine dibutyl and tributyl ether in butanol, 72 g of a 50% aqueous solution of an adduct of hydroabietyl alcohol and 200 moles of ethylene oxide (cross-linked with 1% hexamethylene-1,6-diisocyanate) and 29 g of a 50% aqueous solution of an adduct of hydroabietylamine and 70 moles of ethylene oxide. A finely disperse emulsion is obtained after addition of 389 g of water by stirring.

Resin content: 30%, pH: 4.5.

#### EXAMPLE 6

A mixture of 49 g of an epoxide according to Example 1 (0.25 epoxide equivalent), 27 g of stearylamine (0.1 amino group equivalent) and 10 g of butyl glycol is stirred for 1 hour at 100° C internal temperature. To this mixture are then added 7.8 g of neopentyl glycol (0.15 hydroxy group equivalent) and 11.25 g of anhydrous oxalic acid (0.25 acid equivalent) and stirring is continued for 3 hours at 100° C internal temperature. Then 7 g of epichlorohydrin (0.075 mole) are added and the mixture is stirred for 2 hours at 100° C internal temperature. Subsequently 175 g of an 80% solution of hexamethylolmelamine dibutyl and tributyl ether in butanol, which has previously been diluted with 80 g of butyl glycol, are added dropwise over the course of 30 minutes and stirring is again continued for 30 minutes at 100° C internal temperature. Dilution with 117 g of perchloroethylene yields a clear, 50% solution.

Acid number: 33.2. Viscosity: 6770 cP.

400 g of the above resin solution are mixed with 48 g of a 50% aqueous solution of an adduct of hydroabietyl alcohol and 200 moles of ethylene oxide (cross-linked

with 1% hexamethylene-1,6-diisocyanate) and 19 g of an adduct of hydroabietylamine and 70 moles of ethylene oxide. A finely disperse emulsion is obtained after addition of 533 g of water by stirring.

Resin content: 20%, pH: 3.6.

#### EXAMPLE 7

A mixture of 98 g of an epoxide according to Example 1 (0.5 epoxide equivalent), 31 g of a mixture of 1-aminoeicosane and 1-amino-docosane (0.1 amino group equivalent) and 50 g of dimethyl formamide is stirred for 15 minutes at 100° C internal temperature. To this mixture are then added 15.6 g of neopentyl glycol (0.3 hydroxy group equivalent) and 50.5 g of sebacic acid (0.5 acid equivalent) and stirring is continued for 3 hours at 100° C internal temperature. Subsequently 13.9 g (0.15 mole) of epichlorohydrin are added and stirring is again continued for 3 hours at 100° C internal temperature. Dilution with 159 g of perchloroethylene yields a clear, 50% solution.

Acid number: 27.8. Viscosity: 1400 cP.

300 g of the above resin solution are mixed with 280 g of an 80% solution of hexamethylolmelamine dibutyl and tributyl ether in butanol, 90 g of a 50% aqueous solution of an adduct of hydroabietyl alcohol and 200 moles of ethylene oxide (cross-linked with 1% hexamethylene-1,6-diisocyanate) and 36 g of a 50% aqueous solution of an adduct of hydroabietylamine and 70 moles of ethylene oxide. A finely disperse emulsion is obtained after addition of 6.25 g of diammonium phosphate in 537 g of water by stirring.

Resin content: 30%, pH: 4.9.

#### EXAMPLE 8

A mixture of 49 g of an epoxide according to Example 1 (0.25 epoxide group equivalent) 27 g of stearylamine (0.1 amino group equivalent) and 50 g of butyl glycol is stirred for 1 hour at 100° C internal temperature. To this mixture are then added 7.8 g of neopentyl glycol (0.15 hydroxy group equivalent) and 25.2 g of sebacic acid (0.25 acid equivalent) and stirring is continued for 3 hours at 100° C internal temperature. Subsequently 7 g of epichlorohydrin (0.075 mole) are added and stirring is again continued for 2 hours at 100° C internal temperature.

Then 196 g of an 80% solution of hexamethylolmelamine dibutyl and tributyl ether in butanol are added and stirring is again continued for 1 hour at 100° C internal temperature. Dilution with 183 g of perchloroethylene yields a clear, 50% resin solution.

Acid number: 24. Viscosity: 3570 cP.

500 g of the above 50% resin solution are mixed with 60 g of a 50% aqueous solution of an adduct of hydroabietyl alcohol and 200 moles of ethylene oxide (cross-linked with 1% hexamethylene-1,6-diisocyanate) and 24 g of a 50% aqueous solution of an adduct of hydroabietylamine and 70 moles of ethylene oxide. A finely disperse emulsion is obtained after addition of 668 g of water by stirring. Resin content: 20%, pH: 5.1.

#### EXAMPLE 9

180 g of the 50% resin solution described in Example 7 are mixed with 262 g of an 80% solution of hexamethylolmelamine dibutyl and tributyl ether in butanol, 72 g of a 50% aqueous solution of an adduct of hydroabietyl alcohol and 200 moles of ethylene oxide (cross-linked with 1% hexamethylene-1,6-diisocyanate) and

28 g of a 50% aqueous solution of an adduct of hydroabietylamine and 70 moles of ethylene oxide.

A finely disperse emulsion is obtained after addition of a solution of 4.8 g of diammonium phosphate in 453.2 g of water by stirring.

Resin content: 30%, pH: 4.9.

#### EXAMPLE 10

A mixture of 49 g of an epoxide according to Example 1 (0.25 epoxide equivalent), 27 g of stearylamine (0.1 amino group equivalent) and 50 g of butyl glycol is stirred for 1 hour at 100° C internal temperature. To this mixture are then added 15.2 g of sebacic acid (0.15 acid equivalent) and 4.9 g of maleic anhydride (0.1 acid equivalent) and stirring is continued for 3 hours at 100° C internal temperature. Then 7 g of epichlorohydrin (0.075 mole) are added and stirring is continued for 1 hour at 100° C internal temperature.

Subsequently 174 g of an 80% solution of hexamethylolmelamine dibutyl and tributyl ether in butanol, which has been diluted previously with 50 g of butyl glycol, are added dropwise over the course of 30 minutes and the mixture is stirred for 1 hour at 100° C internal temperature. Dilution with 108 g of perchloroethylene yields a clear, 50% solution.

Acid number: 21.2 Viscosity: 2870 cP.

400 g of the above product are mixed with 48 g of a 50% aqueous solution of an adduct of hydroabietyl alcohol and 200 moles of ethylene oxide (cross-linked with 1% hexamethylene-1,6-diisocyanate) and 19 g of a 50% aqueous solution of an adduct of hydroabietylamine and 70 moles of ethylene oxide. A finely disperse emulsion is obtained after addition of 533 g of water by stirring. Resin content: 20%, pH: 4.9.

#### EXAMPLE 11

With stirring 240 g of the 50% resin solution described in Example 7 are mixed with 224 g of an 80% solution of hexamethylolmelamine dibutyl and tributyl ether in butanol and the mixture is diluted with 136 g of perchloroethylene to give a clear resin solution of medium viscosity.

#### EXAMPLE 12

A mixture of 57.7 g of an epoxide according to Example 1 (0.125 epoxide equivalent), 9.25 g of dodecylamine (0.05 amino group equivalent), 14.45 g of dodecanedicarboxylic acid (0.125 acid equivalent) and 30 g of butyl glycol is stirred for 4 hours at 100° C internal temperature. To this mixture are then added 2 g of acrylonitrile (0.0375 mole) and stirring is again continued for 1 hour at 100° C internal temperature. Subsequently 141.5 g of a 75% solution of hexamethylolmelamine dibutyl and tributyl ether in butanol, which has been diluted previously with 50 g of butyl glycol, are added dropwise and stirring is continued for a further 30 minutes at 100° C internal temperature. The reaction product is then diluted with 74 g of perchloroethylene to give a clear, 50% solution.

Acid number: 17.8. Viscosity: 1080-1070 cP.

200 g of the above product are mixed with 34 g of a 50% aqueous solution of an adduct of hydroabietyl alcohol and 200 moles of ethylene oxide (cross-linked with 1% hexamethylene-1,6-diisocyanate). A finely disperse emulsion is obtained after addition of 99 g of water by stirring. Resin content: 30%, pH: 5.6.

#### EXAMPLE 13

5 A mixture of 49 g of an epoxide according to Example 1 (0.25 epoxide group equivalent), 27 g of stearylamine (0.1 equivalent) and equivalent) and 25 g of butyl glycol is stirred for 1 hour at 100° C internal temperature. To this mixture are then added 8.85 g of 1,6-hexanediol (0.15 hydroxy group equivalent) and 25.2 g of sebacic acid (0.25 acid equivalent) and stirring is continued for 3 hours at 100° C internal temperature. Subsequently 199 g of a 75% solution of hexamethylolmelamine dibutyl and tributyl ether, which has been diluted previously with 60 g of butyl glycol, are added dropwise over the course of 40 minutes and then stirring is continued for a further 30 minutes at 100° C internal temperature. Dilution with 131 g of perchloroethylene yields a clear, 50% resin solution.

Acid number: 24.5. Viscosity: 1080-975 cP.

20 500 g of the above product are mixed with 85 g of a 50% aqueous solution of an adduct of hydroabietyl alcohol and 200 moles of ethylene oxide (cross-linked with 1% hexamethylene-1,6-diisocyanate). A finely disperse emulsion is obtained after addition of 248 g of water by stirring. Resin content: 30%, pH: 4.5.

#### EXAMPLE 14

30 a mixture of 61.25 g of an epoxide according to Example 1 (0.125 epoxide equivalent), 13.5 g of stearylamine (0.05 amino group equivalent) and 25 g of butyl glycol is stirred for 1 hour at 100° C internal temperature. To this mixture are then added 12.6 g of sebacic acid (0.125 acid equivalent) and stirring is continued for a further 3 hours at 100° C internal temperature. After 3.5 g of epichlorohydrin (0.0375 mole) has been 35 added, stirring is continued once more for 2 hours at 100° C internal temperature.

40 A solution of 115 g of hexamethylolmelamine hexamethyl ether in 60 g of butyl glycol is then added dropwise over the course of 30 minutes and stirring is subsequently continued for a further 30 minutes at 100° C internal temperature.

45 Dilution with perchloroethylene yields a clear, 50% resin solution.

Acid number 660 - 541 cP.

50 300 g of the above product are mixed with 52 g of a 50% aqueous solution of an adduct of hydroabietyl alcohol and 200 moles of ethylene oxide (cross-linked with 1% hexamethylene-1,6-diisocyanate). A finely disperse emulsion is obtained by addition of 248 g of water and stirring.

55 Resin content: 25%, pH 4.3.

#### EXAMPLE 15

55 A mixture of 49 g of an epoxide according to Example 1 (0.25 epoxide equivalent), 27 g of stearylamine (0.1 amino group equivalent) and 25 g of butyl glycol is stirred for 1 hour at 100° C internal temperature. To this mixture are then added 15.2 g of sebacic acid (0.15 acid equivalent) and 7.4 g of phthalic anhydride (0.1 acid equivalent and stirring is continued for 3 hours at 100° C. Subsequently 174 g of a 75% solution of hexamethylolmelamine dibutyl and tributyl ether in butanol which has been diluted previously with 50 g of butyl glycol, are added dropwise over the course of 35 minutes and stirring is continued once more for 30 minutes at 100° C. Dilution with perchloroethylene yields a clear, 50% resin solution.

60 Acid number 40.5. Viscosity: 2400-2200 cP.

## 11

450 g of the above product are mixed with 76.5 g of a 50% aqueous solution of an adduct of hydroabietylamine and 200 moles of ethylene oxide (cross-linked with 1% hexamethylene-1,6-diisocyanate).

A finely disperse emulsion is obtained by addition of 5 223.5 g of water and stirring.

Resin content: 30%, pH: 4.8.

## EXAMPLE 16

A mixture of 61.5 g of an epoxide according to Example 1 (0.0625 epoxide equivalent), 6.75 g of stearylamine (0.025 amino group equivalent) and 25 g of butyl glycol is stirred for 1 hour at 100° C internal temperature. To this mixture are then added 1.95 g of neopentyl glycol (0.0375 hydroxy group equivalent) and 6.3 g of sebacic acid (0.063 acid equivalent) and stirring is continued for 1 hour at 100° C internal temperature. Subsequently 132.5 g of a 75% solution of hexamethylolmelamine dibutyl and tributyl ether in butanol, which has been diluted previously with 50 g of butyl glycol, are added dropwise over the course of 30 minutes and stirring is continued for 30 minutes at 100° C internal temperature. Dilution with perchloroethylene yields a clear, 50% resin solution.

Acid number: 15.8. Viscosity: 31520-30500 cP.

200 g of the above product are mixed with 34 g of a 50% aqueous solution of an adduct of hydroabietyl alcohol and 200 moles of ethylene oxide (cross-linked with 1% hexamethylene-1,6-diisocyanate). A finely disperse emulsion is obtained after addition of 166 g of 30 water and by stirring.

Resin content: 25%, pH: 5.4.

## EXAMPLE 17

A mixture of 61.25 g of an epoxide according to Example 1 (0.125 epoxide equivalent), 13.5 g of stearylamine (0.05 amino group equivalent) and 25 g of butyl glycol is stirred for 1 hour at 100° C internal temperature. To this mixture are then added 12.6 g of sebacic acid (0.125 acid equivalent) and stirring is continued for 3 hours at 100° C internal temperature. The 2 g of acrylonitrile (0.0375 mole) are added and the mixture is stirred for 1 hour at 100° C internal temperature. Subsequently 152 g of a 75% solution of hexamethylolmelamine dibutyl and tributyl ether in butanol, which has been diluted previously with 65 g of butyl glycol, are added dropwise over the course of 30 minutes and stirring is continued for a further 30 minutes at 100° C internal temperature. Dilution with 75 g of perchloroethylene yields a clear, 50% resin solution.

Acid number 27.6. Viscosity: 5400 cP.

300 g of the above product are mixed with 52 g of a 50% aqueous solution of an adduct of hydroabietyl alcohol and 200 moles of ethylene oxide (cross-linked with 1% hexamethylene-1,6-diisocyanate). A finely disperse emulsion is obtained after addition of 248 g of 55 water and by stirring.

Resin content: 25%, pH: 5.0.

## EXAMPLE 18

## a. Opaque dressing on box calf leather

200 parts of an iron oxide dispersion (30% pigment content) are mixed with 450 parts of the emulsion according to Example 1 and subsequently diluted with water to 1000 parts. The pigmented finishing solution is sprayed 4 times crosswise on box calf leather. The leather is then dried and subsequently sprayed twice cross-wise with a colourless finishing solution of

## 12

450 parts of the emulsion according to Example 1

10 parts of phosphoric acid and

490 parts of water

at 25° C to 30° C. The leather is then dried for 2 hours

at 60° C and ironed at 80° C/100 bar.

b. Box calf leather is sprayed on both sides with the colourless finishing solution according to (a) and then dried. The finished leather has a good microbiocidal action both on its top side (finish a) and on both sides (finish b) in the tests as described in below. Moreover, the leather is provided with a finish which is fast to light and rubbing. It has good crease resistance and is stable to ironing up to 250° C.

Analogous results are obtained with the emulsions according to Examples 2 to 17.

These finished leather samples are tested in the agar diffusion test (AATCC test method 90-1970, modified) and in the disinfection test (AATCC test method 100-1970, modified) for their resistance to the following test organisms:

bacteria:

Staphylococcus aureus SG 511

Escherichia coli NCTC 8196

Proteus vulgaris NCIB 4175

fungi:

Trichophyton mentagrophytes ATCC 9533

## 1. Agar diffusion test (inhibition test).

Test samples in the form of round discs measuring 2 cm in diameter are punched from the finished leather. Sterile AATCC bact. Agar BBL (5ml) is then poured into a petri dish. After the agar layer has set, the test samples are laid in the dish with their top sides resting on this agar layer. Then 10 ml of the same nutrient medium, which is inoculated with test microorganisms, is poured over the samples.

The inoculation is effected by adjusting overnight cultures of the test microorganisms in Difco brain-heart-infusion broth by dilution with sterile broth in such a way that, after addition of the inoculum to the agar, the concentration of the microorganisms is  $5 \cdot 10^5 - 1 \cdot 10^6$  per ml of agar. The dishes are then incubated for 24 hours at 37° and the inhibition zones are subsequently read off.

A similar procedure is carried out with the test microorganism Trichophyton mentagrophytes ATCC 9533. The deviations from the described procedure are:

The inoculum is prepared by elutriating an at least 7 day old slant agar culture on Mycosel Agar BBL with 10 ml of Mycophil Broth BBL, filtering it through sterile glass wool and adding it to the agar. The microorganism concentration is adjusted to about  $5 \cdot 10^4 - 1 \cdot 10^6$  spores per ml of agar. The test nutrient medium used in the petri dish for Trichophyton was Mycosel Agar BBL. These dishes are incubated for 7 days at 28° C.

## 2. Disinfection Test

60 Test samples in the form of round discs (diameter 2 cm) are punched from the leather under investigation and sterilised with ethylene oxide. The sterilised samples are then inoculated with the test microorganisms using 10 drops of a suspension per sample. The suspension for the inoculum is prepared in the same way as that described for the agar diffusion test and by diluting in such a way that in the end effect the following microorganism concentrations are present on the test sam-

ples: bacteria  $10^6$  –  $10^7$  microorganisms per sample and Trichophyton app.  $5 \cdot 10^5$  spores per sample.

The inoculated samples are put into a humid chamber and incubated for 24 hours at  $37^\circ\text{C}$  (for Trichophyton at  $28^\circ\text{C}$ ). Following the incubation in the humid chamber, the samples are extracted in 20 ml of phosphate buffer (pH 7.4) with the addition of 1% TWEEN-80. After the extraction, 1 ml at a time of the solution is mixed with 9 ml of AC-Agar Difco or Myco-sel Agar Difco (for Trichophyton) and poured into dishes. For the agar, 1% TWEEN-80 is once again added as blocking agent. These dishes are incubated for 24 hours at  $37^\circ\text{C}$  (in the case of Trichophyton for 7 days at  $28^\circ\text{C}$ ). The germ counts are then taken, comparisons are made with corresponding controls, and any microstatic after-effects in the dishes (as a consequence of insufficient blocking) are prevented by reinoculation.

The described tests are used to determine whether the test microorganisms are inhibited in their growth (microbiostatic effect) or whether they are destroyed (microbiocidal effect).

The finished leather samples exhibit good antimicrobial effects (very good action against Trichophyton — fungistatic and fungicidal — as well as good action against bacteria — microbiostatic and microbiocidal).

d. Fastness to wet rubbing: the finished leather is rubbed 150 times in two directions with a moist piece of wool felt while applying pressure (1 bar gauge).

e. Crease resistance: In this test, the finished leather is creased 50,000 times and inspected in order to determine whether and/or to what extent the finish (outermost layer) has been impaired at the creases.

f. Resistance to ironing: The finished leather is ironed at  $250^\circ\text{C}$  and inspected in order to determine whether and/or to what extent the finish melts.

The results of tests (d) to (f) are reported in a rating from 1 to 5, with 5 being the highest rating.

g. Results: (Dressing of leather in accordance with (a))

| preparation according to | fastness to wet rubbing | crease resistance | resistance to ironing |
|--------------------------|-------------------------|-------------------|-----------------------|
| Example 1                | 5                       | 4 – 5             | 5                     |
| 2                        | 4 – 5                   | 4                 | 4 – 5                 |
| 3                        | 5                       | 4 – 5             | 5                     |
| 4                        | 3 – 4                   | 4                 | 4                     |
| 6                        | 4 – 5                   | 4                 | 4 – 5                 |
| 12                       | 5                       | 4 – 5             | 5                     |
| 13                       | 5                       | 4 – 5             | 5                     |
| 14                       | 5                       | 4 – 5             | 5                     |
| 15                       | 5                       | 4 – 5             | 5                     |
| 16                       | 5                       | 4 – 5             | 5                     |
| 17                       | 5                       | 4 – 5             | 5                     |

We claim:

1. A process for dressing and providing leather with an antimicrobial finish which comprises treating the leather with aqueous or organic preparations of

1. reaction products of

- an epoxide that contains at least two epoxide groups in each molecule,
- a fatty amine with 12 to 24 carbon atoms,
- a dicarboxylic acid of the formula



wherein  $y$  is an integer from 1 to 13, optionally

d. an anhydride of an aromatic dicarboxylic acid with at least 8 carbon atoms, of an aliphatic monocarboxylic acid with at least 2 carbon atoms, or of an aliphatic dicarboxylic acid with at least 4 carbon atoms,

e. an aliphatic diol with 2 to 21 carbon atoms and/or

f. a difunctional compound which differs from components (a), (c), (d) and (e), which reaction products have been reacted or mixed or reacted and mixed with

2. aminoplast precondensates which contain alkyl ether groups, and subsequently drying the treated leather at elevated temperature.

3. A process according to claim 1, which comprises treating the leather with preparations of reaction products of components (a), (b), (c), (d), (e), (f) and (2).

4. A process according to claim 1, which comprises treating the leather with preparations of mixtures of reaction products of components (a), (b), (c), (d), (e) and (f); (a), (b), (c) and (e) or (a), (b), (c) and (f) and component (2).

5. A process according to claim 1, which comprises treating the leather with preparations of reaction products in which the component (a) is an epoxide which is derived from a bisphenol.

6. A process according to claim 5, which comprises treating the leather with preparations of reaction products in which the component (a) is a polyglycidyl ether of 2,2-bis-(4'-hydroxyphenyl)-propane with an epoxide content of 1 to 6 epoxide group equivalents per kilogram.

7. A process according to claim 5, which comprises treating the leather with preparations of reaction products in which the component (a) has an epoxide of at least 5 epoxide group equivalents per kilogram.

8. A process according to claim 5, which comprises treating the leather with preparations of reaction products in which the component (a) is a reaction product of epichlorohydrin and 2,2-bis-(4'-hydroxyphenyl)-propane.

9. A process according to claim 1, which comprises treating the leather with preparations of reaction products in which the component (b) is a mono-fatty amine with 16 to 22 carbon atoms.

10. A process according to claim 1, which comprises treating the leather with preparations of reaction products in which the component (c) is a dicarboxylic acid of the formula



55

wherein  $y$  is a whole number from 6 to 13.

11. A process according to claim 1, which comprises treating the leather with preparations of reaction products in which the component (d) is an anhydride of a 60 monocyclic or bicyclic aromatic dicarboxylic acid with 8 to 12 carbon atoms or of an aliphatic dicarboxylic acid with 4 to 10 carbon atoms.

12. A process according to claim 1, which comprises treating the leather with preparations of reaction products in which the component (d) is an anhydride of a 65 monocarboxylic acid with 2 to 10 carbon atoms.

13. A process according to claim 11, which comprises treating the leather with preparations of reaction

15

products in which the component (d) is an anhydride of a monocyclic aromatic dicarboxylic acid with 8 to 10 carbon atoms.

14. A process according to claim 13, which comprises treating the leather with preparations of reaction products in which the component (d) is a phthalic anhydride which is optionally substituted by methyl.

15. A process according to claim 1, which comprises treating the leather with preparations of reaction products in which the component (e) is an aliphatic diol with 2 to 6 carbon atoms the carbon chain of which is optionally interrupted by oxygen atoms.

16. A process according to claim 15, which comprises treating the leather with preparations of reaction products in which the component (e) is an alkylene diol with 2 to 6 carbon atoms or is diethylene or triethylene glycol.

17. A process according to claim 1, which comprises treating the leather with preparations of reaction products in which the component (f) is a difunctional organic compound which contains as functional groups or atoms halogen atoms bonded to an alkyl radical, vinyl groups or carboxylic acid ester groups or at most one epoxide, carboxy or hydroxy group together with another functional group or another atom of the indicated kind.

18. A process according to claim 17, which comprises treating the leather with preparations of reaction products in which the component (f) is a difunctional organic compound which contains as functional groups or atoms chlorine or bromine atoms bonded to an alkyl radical, vinyl groups or carboxylic acid alkyl ester groups or at most one epoxide or carboxy group together with another functional group or another atom of the indicated kind.

19. A process according to claim 18, which comprises treating the leather with preparations of reaction products in which the component (f) is an epihalohydrin.

20. A process according to claim 1, which comprises treating the leather with preparations of reaction products in which the component (2) is an alkyl ether of

16

methylolated urea, methylolated urea derivatives or, preferably, of methylolated amino-triazines.

21. A process according to claim 20, which comprises treating the leather with preparations of reaction products in which the component (2) is an alkyl ether of a highly methylolated melamine the alkyl radicals of which contain 1 to 4 carbon atoms.

22. A process according to claim 21, which comprises treating the leather with preparations of reaction products in which the component (2) contains a n-butyl ether of a highly methylolated melamine which contains 2 to 3 n-butyl radicals in the molecule.

23. A process according to claim 1, which comprises treating the leather with preparations of reaction products or mixture of (1) 1 epoxide equivalent of component (a), 0.05 to 0.7 amino group equivalent of component (b), 0.2 to 2.0 acid equivalents of component (c) and (d), optionally 0.1 to 0.8 hydroxy group equivalent of component (e), 0.1 to 0.7 mole of component (f) and 10 to 80 percent by weight of component (2), based on the total weight of components (a) to (f) and (2) or on the weight of the mixture of (1) and (2), the components (2) being used as reaction component or as mixture component or as both.

24. A process according to claim 23, which comprises treating the leather with preparations of mixtures of (1) and (2) in a weight ratio of (90 to 20); (10 to 80).

25. A process according to claim 1, which comprises the use of aqueous solutions or emulsions as preparations.

26. A process according to claim 1, which comprises treating the leather at 20° to 100° C, preferably at room temperature.

27. A process according to claim 1, which comprises drying the treated leather at 100° to 160° C, preferably at 120° to 140° C.

28. The leather which is dressed and provided with an antimicrobial finish according to the process of claim 1.

\* \* \* \* \*

45

50

55

60

65

UNITED STATES PATENT AND TRADEMARK OFFICE  
CERTIFICATE OF CORRECTION

PATENT NO. : 3,991,238

DATED : November 9, 1976

INVENTOR(S) : ROSEMARIE TÖPFL ET AL

It is certified that error appears in the above-identified patent and that said Letters Patent are hereby corrected as shown below:

In column 16, claim 27, lines 37 and 38, change  
"100° to 160°C, preferably at 120° to 140°C" to  
-- 40° to 70°C --.

Signed and Sealed this

First Day of February 1977

[SEAL]

Attest:

RUTH C. MASON  
*Attesting Officer*

C. MARSHALL DANN  
*Commissioner of Patents and Trademarks*